

Oct. 9, 1923.

1,469,824

P. C. SEEL

PROCESS OF PREPARING ALKALI CELLULOSE

Filed Jan. 27, 1923

FIG - 1.



FIG - 2.



FIG - 3.



FIG - 4.



INVENTOR.

Paul C. Seel,  
BY R. L. Stinchfield

ATTORNEY

Patented Oct. 9, 1923.

1,469,824

# UNITED STATES PATENT OFFICE.

PAUL C. SEEL, OF ROCHESTER, NEW YORK, ASSIGNOR TO EASTMAN KODAK COMPANY, OF ROCHESTER, NEW YORK, A CORPORATION OF NEW YORK.

## PROCESS OF PREPARING ALKALI CELLULOSE.

Application filed January 27, 1923. Serial No. 615,414.

*To all whom it may concern:*

Be it known that I, PAUL C. SEEL, a citizen of the United States of America, residing at Rochester, in the county of Monroe and State of New York, have invented certain new and useful Improvements in Processes of Preparing Alkali Cellulose, of which the following is a full, clear, and exact specification.

10 This invention relates to processes of preparing alkali celluloses, particularly those types which are suitable for the preparation of cellulose ethers. One object of the invention is to provide simple and reliable 15 processes. Other objects will hereinafter appear.

In the accompanying drawing, which forms a part hereof:

20 Fig. 1 is a diagrammatic sectional view of a ball mill in which the first step of the preferred form of my process may be carried out;

25 Fig. 2 is a similar section of the same mill showing the condition of the material at the end of the first step;

Fig. 3 is a diagrammatic sectional view of the mill illustrating another step in the process, and

30 Fig. 4 is a diagrammatic sectional view of the mill showing the final step of the process.

In the preparation of cellulose ethers it has been found that the possibility of obtaining products having the desired characteristics depends to an unexpected degree upon the manner and thoroughness with which the ingredients of the alkali cellulose are mixed. For example, if the ethers derived from improperly mixed alkali cellulose be used in the making of films, the latter will exhibit a very undesirable haze. I have discovered a simple and reliable method of effecting the mixture of the ingredients in the alkali cellulose to such an extent that this haze is practically eliminated from ethers derived from it.

40 A mass of cellulose fibers, alkali and water in the proportions desirable for subsequent etherification is not easy to handle by means of ordinary grinding, because it clumps up into a resistant mass. I have found, however, that if a rough or incomplete mixture of the ingredients in the desired proportions be first formed into a large number 55 of small compacted dense masses or units

and then these be pulverized, the action is simple to carry through completely.

The preferred form of my invention will be described by way of illustration, but the invention is not limited thereto, except as indicated in the appended claims. Referring to Fig. 1 the materials 1 to be mixed in the form of alkali cellulose are charged into a cylindrical ball mill 2, along with the grinding elements or balls 3, access to the interior being had through the normally closed door 4. The charge may, for example, be 100 parts of cotton or wood cellulose or cellulose tissue, together with 200 parts of solid caustic soda and 250 parts of water.

With the door 4 closed the ball mill is then rotated, as will be readily understood by those skilled in the art. The balls 3 do not, as might have been expected, grind up and entirely mix the material. Instead, they only roughly mix the materials and clump or compact them into a dense mass which lines the ball mill 2 and the cover 4. There may be also a dense lining on some or all of the balls. This is indicated diagrammatically in Fig. 2, the compacted mass being shown at 11.

As indicated in Fig. 3, the cover 4 is removed along with the balls and the interior lining or compacted mass 11 is broken up into small compacted dense pieces or units 5 by any suitable tool or instrument 6. Of course, any material which has been compacted on the surfaces of the balls 3 and door 4 may be similarly scraped or broken up.

The small compacted dense masses or clumps thus obtained are charged with the balls 3 again into the mill 2. The door 4 is closed and the mill rapidly rotated. The compacted masses are then rapidly and thoroughly pulverized and the ingredients thereby are brought to the intimate state of admixture which is so essential for the best production of cellulose ethers.

The etherification is, of course, carried out in any of the known or preferred ways. An alkali cellulose having the ingredients in the illustrative proportions mentioned above may be charged into an autoclave with 400 parts of ethyl chloride for each 100 parts of cellulose in the mixture. The autoclave can then be heated for say twenty-four hours at temperatures between 90° and 170° C.

Having thus described my invention, what I claim as new and desire to secure by Letters Patent is:

1. The process of preparing pulverulent intimately mixed alkali cellulose which comprises the steps of forming the ingredients, including the cellulose and alkali, into small compacted dense masses and then pulverizing said masses.
- 10 2. The process of preparing pulverulent intimately mixed alkali cellulose which comprises the steps of forming the ingredients, including the cellulose and alkali, into a compacted dense mass, dividing said mass into a plurality of small dense masses, and then pulverizing said small masses.
- 15 3. The process of preparing pulverulent

intimately mixed alkali cellulose suitable for etherification, which comprises the steps of first agglomerating caustic alkali, cellulose, and water into dense compacted small units and then reducing said units to powder.

20 4. The process of preparing pulverulent intimately mixed alkali cellulose, suitable for etherification, which comprises the steps of compacting caustic soda, cellulose, and water into a dense layer, breaking up said layer into fragments, and then grinding said fragments to powder.

25 Signed at Rochester, New York this 20th day of January 1923.

30 PAUL C. SEEL.